

Nov. 23, 1937.

F. C. KELLEY

2,100,218

METER PIVOT

Filed June 20, 1935



Inventor:  
Floyd C. Kelley,  
by *Harry E. Dunham*  
His Attorney.

## UNITED STATES PATENT OFFICE

2,100,218

## METER PIVOT

Floyd C. Kelley, Schenectady, N. Y., assignor to  
General Electric Company, a corporation of  
New York

Application June 20, 1935, Serial No. 27,615

5 Claims. (Cl. 308—159)

The present invention relates to pivots and more particularly to pivots which are adapted for use in measuring instruments such as watt hour meters and like devices.

5 Heretofore pivots employed in such devices generally have been made of steel, the pivots being about 37 mils in diameter and having a bearing end with a radius of about 18½ mils. Such pivots are entirely satisfactory from the stand-  
10 point of hardness and resistance to impact but when employed in meters which are exposed to the elements and particularly to salt air conditions the pivots quickly corrode. The resultant oxide coating on the pivots slows down the meter  
15 and may even cause it to stick and fail to operate.

It is an object of the present invention to provide a meter pivot which has a satisfactory degree of hardness and which resists impact.

20 The novel features which are characteristic of my invention are set forth with particularity in the appended claims. The invention itself, however, will best be understood from reference to the following specification when considered in  
25 connection with the accompanying drawing in which the single figure is a view on an enlarged scale partly in section and partly in elevation of a meter pivot embodying the features of my invention.

30 Referring more particularly to the drawing, I have indicated at 1 a pivot assembly of the character generally employed in watt hour meters. It comprises a pivot member 2 supported on a sapphire bearing 3. The pivot 2 is rounded at each end and carries a shaft 4 at its upper end. The lower portion of the pivot extends through a  
35 guide bushing 5 which holds a lubricant 6 which is supplied to the bearing 3.

In carrying out my invention, I employ as the  
40 pivot 2 a precipitation or age hardened cobalt tungsten alloy such as disclosed in the copending Sykes application Serial No. 525,025, filed May 24, 1931, and assigned to applicant's assignee. The alloy may be fabricated in the manner dis-  
45 closed in the Sykes application either by casting the alloy and then heat treating it as hereinafter disclosed or by fabricating the alloy from powdered ingredients. In the latter case about 20 to 35% of powdered tungsten is mixed with about  
50 80 to 65% of powdered cobalt. The mixed materials are pressed into a desired shape and sintered at an elevated temperature in an inert or suitable reducing atmosphere such as hydrogen. The sintering may be carried out at temperatures above

1100° C., for example about 1400 to 1450° C. and the sintering period employed will vary with the temperature employed. The alloy may be quenched or cooled slowly from the sintering temperature after which it is aged or precipita-  
5 tion hardened by heating at a temperature between about 500 and 800° C. for a period of time varying from about 20 to 100 hours.

The alloy offers a high resistance to impact and the products of corrosion, unlike the products of 10 corrosion of steel, are non-abrasive. It prefer-  
ably should be carbon free but a small amount of carbon, for example .05% does not materially affect the hardness of the alloy. However, if the carbon content is as high as .20% the hard-  
15 ness of the alloy is noticeably lessened.

Although I prefer to employ an age hardened alloy consisting of cobalt and tungsten, as hereinbefore set forth, my invention is not limited to the use of that alloy. Other age hardened alloys, 20 for example cobalt-molybdenum, nickel-molyb-  
denum or alloys consisting of about 20% to 35% of metal from a group consisting of tungsten and molybdenum with about 80% to 65% of metal from a group consisting of cobalt and nickel, 25 may be employed if desired, although it will be found that the best results are obtained with the cobalt-tungsten alloy having a composition such as hereinbefore set forth.

What I claim as new and desire to secure by 30 Letters Patent of the United States is:

1. A pivot consisting substantially of about 20% to 35% of metal from a group consisting of tungsten and molybdenum and about 80% to 65% of metal from a group consisting of cobalt and 35 nickel.

2. An age hardened meter pivot consisting sub-  
stantially of about 20% to 35% of metal from a group consisting of tungsten and molybdenum and about 80% to 65% of metal from a group con-  
40 sisting of cobalt and nickel.

3. A meter pivot consisting substantially of about 20% to 35% tungsten and about 80% to 65% cobalt.

4. An age hardened meter pivot consisting sub-  
stantially of about 20% to 35% tungsten and about 80% to 65% cobalt.

5. In combination, a bearing member, a rotat-  
ing member cooperating therewith, one of said  
members consisting of an age hardened alloy con-  
taining about 20% to 35% tungsten and about  
80% to 65% cobalt.

FLOYD C. KELLEY.